

## UNITED STATES PATENT OFFICE

MORTIMER T. HARVEY, OF NEWARK, NEW JERSEY, ASSIGNOR TO THE HARVEL CORPORATION, OF NEWARK, NEW JERSEY, A CORPORATION OF NEW JERSEY

## CONTAINER AND MATERIAL THEREFOR

No Drawing. Original application filed October 1, 1927, Serial No. 223,481. Divided and this application filed October 21, 1927. Serial No. 227,862.

The present invention relates to containers and to material for containers with which are associated a coating or an impregnation of a material made from the oil or liquid which occurs in the cellular outer shell or husk of the cashew nut and to method of producing these products. Containers having such a coating thereon or impregnated therewith are particularly useful for holding and transporting foodstuffs because this material is insoluble in water, alcohol, oils, dilute acids and alkalis, and other solvents; and for this reason such containers are useful for holding dilute acids or alkalis, ether, alcohol, oils, and so on, and the materials and the containers made according to the invention are useful in the arts generally.

Various objects and advantages of the invention will be obvious from the following description of new and useful containers and container material embodying the invention; and the invention consists of the containers and container material set forth in the claims.

The material for coating the containers of the invention and for impregnating the same or others thereof is made by treating the oil or liquid from the husk of the cashew nut to make it insoluble when dried and also to make it presentable either by itself or by means of a carrier vehicle or by a solvent to apply it to a material to be coated or impregnated or both as by flowing or dipping or brushing or other suitable methods or means.

The methods of making the oil insoluble are set forth in various copending applications but two suitable examples will be cited here to make the present invention practicable. One method is to heat the husk oil of the cashew nut in contact with copper metal at a temperature of about 200° C. for about forty-five minutes at normal pressure. The resultant material is a liquid which itself can be applied to a surface by some of the methods above cited. This resultant liquid can also be taken up with a solvent such as kerosene, naphtha, benzine or the like. In either case, whether applied by itself or by a solvent or other vehicle the reaction product, after removing the vehicle in cases where used, will dry to a tough, resilient or flexible

body or film. A suitable temperature for drying the reaction product is 104° C. for an hour and in some cases for very much less time.

For some purpose gelled linseed oil is mixed with the above reaction product and applied as by means of a solvent vehicle. This is desirable for example when the cashew shell oil is limited in quantity and linseed oil not so limited. The product involving linseed oil has many of the desirable characteristics of the product of the cashew shell oil alone although in some cases not to the same degree. These coating materials as well as the others herein noted are among other uses notably suited for lining bottle caps and caps for other containers, for example, for mustard and pickle bottles, for cardboard ice cream containers, and lining the caps on metal bottles for containing ether. The characteristics which make these products suitable for the particular purposes above noted are insolubility, freedom from taste and smell and proof against dampness and absorption of water.

Another method of producing coating and impregnating material for containers is substantially as follows. The cashew nut shell oil is heated with about 10% of its weight of nitric acid sp. gr. 1.40 for about thirty minutes at a temperature of about 240° C. The reaction product is washed to free it of acid and is taken up with a vehicle such as kerosene. The application of this form is by dipping, brushing, or spraying as with the others.

The materials for making containers for which the above described reaction products of cashew nut husk oil are any of the materials heretofore used such as paper, cardboard, wood, gelatines, cellulose acetate and the like, metal and other material some not heretofore used because of unsuitability on account of porousness, absorption of moisture, and other reasons. The material named can be rendered gas tight by a coating of one of the reaction products named. These products can be used also for waterproofing or moisture proofing wood, paper, glacine paper, cellulose products and so on.

Food containers in particular can be made of material which has been impregnated or coated with the reaction products named.

A further use for the material is the replacement of tin for coating iron in the making of sheet metal containers, the material being peculiarly adapted for this use because of its insolubility in food juices, certain acids and alkalis, acetic acid-brine pickling solutions, and hydrocarbons which are generally known as solvents such as kerosene, gasoline and the like. The material can be used for coating copper and the copper which is coated can be utilized for bringing the cashew oil into a condition in which it will dry as for example according to the copper reaction above described. In the making containers either or both the inside and the outside surface of the container is or are provided with the coating described. Also the material for the container is coated either before or after the container is made thereof.

A still further method of making containers or container material is to produce a thin coating of copper on sheet iron as by immersing the sheet iron in a copper sulphate bath until the iron becomes coated with the copper, or by electrolytic deposition with electrodes. The copper coating on the iron is then utilized to catalyse a reaction of cashew nut shell liquid brought in contact therewith. In making metal containers or in making the material therefor a coating of cashew nut shell liquid varnish can be obtained by immersing the material of the container itself in the shell liquid which is at a temperature of about 200° C. for about forty-five minutes after which the immersed and treated material is withdrawn from the bath and properly drained to secure an even coating of the treated liquid therewith. Further heating at from 100° to 150° C. or more is then used to set the resultant coating on the surface. A still further method of preparing the cashew nut shell liquid for making the coating or impregnating material is to heat it up to about 600° F. and then allow it to cool. Dryers such as litharge, or manganese dioxide, or copper oleate, or mixtures of these, or other driers, can be added at suitable temperatures; 450° F. is a practical temperature for adding the driers. The treated liquid, with or without the drier, can be applied with or without a solvent as a coating or impregnation and dried at say about 100° to 125° C. for examples. Also linseed oil, China wood oil, gums, or resins or mixtures of these can be added to the cashew nut shell liquid before or after or part before and part after the treatment of the cashew liquid and in these cases the drier can be used or not, to secure different results.

Although I have set forth and described various methods and processes for producing

my new products, it is obvious that various changes may be made in the methods or processes or in the various steps thereof without changing or modifying the essential features and characteristics of the products produced and that such products remain substantially with the same desirable characteristics although modifications may be made in the appearance, texture and in the physical and chemical characteristics. 75

As to certain features claimed in the present application, the present application constitutes a division of my copending application Serial No. 223,481, filed October 1, 1927. 80

The various methods above referred to for making cashew nut shell liquid insoluble are set forth in my Patents Nos. 1,725,791; 1,725,792; 1,725,793; 1,725,794; 1,725,795; 1,725,796; and 1,725,797; all issued August 27, 1929, the application for each of which was copending with the present application. 85

What I claim as new and desire to secure by Letters Patent is:

1. A web of fibrous material which has on the surface thereof a coating which has modified cashew nut shell liquid as the base thereof. 90

2. A container having a wall of fibrous material which has on the surface thereof a coating which has modified cashew nut shell liquid as the base thereof. 95

3. A web of fibrous material which has on the surface thereof and is impregnated with a material which has modified cashew nut shell liquid as the base thereof. 100

4. A container having a wall of fibrous material which has on the surface thereof and is impregnated with a material which has modified cashew nut shell liquid as the base thereof. 105

5. A container having a wall of fibrous material which has on its inner surface a coating which has modified cashew nut shell liquid as the base thereof. 110

6. A container having a wall of fibrous material which is impregnated with and is coated on its inner surface with a material which has modified cashew nut shell liquid as the base thereof. 115

7. A container having a wall of fibrous material which is impregnated with and is coated on its inner and outer surfaces with a material which has modified cashew nut shell liquid as the base thereof. 120

8. Cardboard which has on the surface thereof a coating which has modified cashew nut shell liquid as the base thereof.

9. Cardboard which has on the surface thereof and is impregnated with a material which has modified cashew nut shell liquid as the base thereof. 125

10. A container having a wall of cardboard which has on the surface thereof a coating 130

which has modified cashew nut shell liquid as the base thereof.

11. A container having a wall of cardboard which has on the surface thereof and is impregnated with a material which has modified cashew nut shell liquid as the base thereof.

12. A web of cellulose material having on the surface thereof a coating which has modified cashew nut shell liquid as the base thereof.

13. A container having a wall of cellulose material which is coated with and is impregnated with a material which has modified cashew nut shell liquid as the base thereof.

14. A web of fibrous material which has on the surface thereof and is impregnated with cashew nut shell liquid modified to a dry state.

15. A web of cardboard which has on the surface thereof and is impregnated with cashew nut shell liquid modified to a dry state.

16. A web of fibrous material impregnated with cashew nut shell liquid modified to a dry state.

17. A web of cardboard impregnated with cashew nut shell liquid modified to a dry state.

18. A web of fibrous material having between the fibers thereof cashew nut shell liquid modified to a dry state.

19. A container which has a coating on the surface thereof of modified cashew nut shell liquid.

20. A container having on the wall thereof a coating which is a varnish made from cashew nut shell liquid.

21. A container having on the surface thereof a coating of modified cashew nut shell liquid which is resistant to the action of food juices.

In testimony, that I claim the invention set forth above I have hereunto set my hand this 28th day of September, 1927.

**MORTIMER T. HARVEY.**